

1

3,155,615

SOLS OF METAL DIALKYL DITHIOPHOSPHATES  
 Elmer B. Cyphers, Cranford, N.J., assignor to Esso Research and Engineering Company, a corporation of Delaware  
 No Drawing. Filed Aug. 1, 1961, Ser. No. 128,368  
 10 Claims. (Cl. 252—32.7)

This invention relates to colloidal sols containing metal dialkyl dithiophosphates, methods for their preparation and their use. Particularly, the invention relates to metal salts of low molecular weight dialkyl dithiophosphates prepared by neutralizing dialkyl dithiophosphoric acid in the presence of a detergent additive.

The use of metal dialkyl dithiophosphates as lubricating oil additives is well known in the art. These materials are commercially used on a wide scale because of their excellent properties in imparting extreme pressure, anti-wear and rust prevention properties to mineral lubricating oil. The active portions of the metal dialkyl dithiophosphates are the metal, the phosphorus and the sulfur, while the dialkyl group primarily serves the purpose of solubilizing the material into the mineral oil. From an economic and efficiency standpoint, it is highly desirable to make the dialkyl groups as small as possible and still retain oil solubility. Normally, dialkyl dithiophosphates having alkyl groups containing less than 6 carbon atoms are insoluble in the mineral oil. However, it has recently been found that, by using certain select mixtures of dialkyl groups of different carbon atom content, alkyl groups averaging less than 6 carbon atoms can be used. One such dithiophosphate is prepared from mixed C<sub>4</sub> and C<sub>5</sub> alkyl groups, while another is prepared from mixed C<sub>3</sub> and C<sub>6</sub> alkyl groups. However, it has not heretofore been possible to prepare a stable oil solution of metal dialkyl dithiophosphate wherein the alkyl groups have an average carbon atom content of three or less. The present invention is based upon the discovery that stable oil compositions containing dialkyl dithiophosphates can be made where each alkyl group contains 3 carbon atoms or less, and which are effective as lubricating oil additives. Furthermore, the dithiophosphates of the invention are more effective than the present commercially available dithiophosphates since by preparing the salt from lower molecular weight dialkyl groups, then a given pound of material will contain a larger proportion of the metal, phosphorus and sulfur which are the effective portions of the molecule.

The metal dialkyl dithiophosphates of the invention are those wherein each alkyl chain contains 1 to 3 carbon atoms, while the metal may be any metal which forms a water-insoluble dialkyl dithiophosphate, for example: zinc, lead, cadmium, molybdenum, etc. Specific examples of such dithiophosphates are zinc dimethyl dithiophosphate, lead diethyl dithiophosphate, cadmium methyl-ethyl dithiophosphate, molybdenum di-isopropyl dithiophosphate, etc.

In order to obtain the colloidal sols of the dialkyl dithiophosphates of the invention it is necessary that said dithiophosphates be prepared in the presence of a detergent additive. In general, additives soluble in the oil and having good dispersing or detergent properties will be operable. However, it is preferred to use those detergents which are lubricating oil detergents since such detergents serve the additional function of maintaining cleanliness of the lubricated parts, e.g., automotive engines.

The detergent additives which are preferred include petroleum sulfonates, synthetic alkyl aryl sulfonates, various alkyl phenates, alkyl phenate sulfides, phosphosulfurized olefin polymers, and various combinations of these additives. Following are specific descriptions of several of the above types of detergent additives.

2

Petroleum sulfonates generally used as lubricating oil detergents are the oil-soluble alkaline earth metal salts of high molecular weight sulfonic acids. These sulfonic acids are produced by the treatment of petroleum oils of the lubricating oil range with fuming sulfuric acid and generally have molecular weights of about 300 to 700 e.g., 350 to 500. Petroleum sulfonates are well known in the art and have been described in numerous patents, e.g., U.S. 2,467,176.

10 Detergent sulfonates can also be derived synthetically from relatively pure alkyl aryl sulfonic acids having from about 10 to 33 carbon atoms per molecule. For example, sulfonated products of alkylated aromatics such as benzene, toluene, xylene, and naphthalene, alkylated with olefins or olefin polymers of the type of polypropylene, polyisobutylene, etc. can be used.

Specific examples of the above two types of sulfonates include calcium petroleum sulfonate, barium petroleum sulfonate, calcium di-C<sub>8</sub> alkyl benzene sulfonate, barium di-C<sub>9</sub> alkyl benzene sulfonate and calcium C<sub>16</sub> alkyl benzene sulfonate; wherein said di-C<sub>8</sub> alkyl group is derived from diisobutylene; said C<sub>9</sub> alkyl group is obtained from tripropylene and said C<sub>16</sub> alkyl group is obtained from triaisobutylene.

25 The above sulfonates may be either neutral sulfonates, i.e., where the sulfonic acid is neutralized with an equal mole equivalent amount of metal base, or the sulfonates may be of the so-called "high alkalinity" type. In the latter case, additional metal base, in excess of that required for simple neutralization, is reacted with the sulfonate sulfonic acid to form an alkaline product which can then be blown with carbon dioxide to reduce its alkalinity and form a substantially neutral final product. Recent work has indicated that such so-called high alkalinity sulfonates are nothing more than dispersions of neutral sulfonates and a carbonate of the metal used which are believed to exist in the form of colloidal sols. In any event, the term sulfonate as used herein and in the appended claims includes both neutral sulfonates and so-called high alkalinity (or high metal content) sulfonates.

30 Phenate sulfides are also well known in the art and have been described in numerous patents, for example, U.S. 2,451,345 and U.S. 2,362,289. The more important of these materials are metal salts of phenol sulfides which may be typified by the following formula:



wherein R represents an alkyl group, a is 0 to 4, b is 0 to 10 and c is 1 to 5. The metal used to form the phenate may be aluminum, cobalt, chromium, sodium, lead, tin, etc., or the alkaline earth metals as calcium, barium, strontium and magnesium. Each alkyl group can contain 5 to 20, e.g., 7 to 12 carbon atoms, either straight or branched chain. Specific examples of the phenate sulfides include barium tertiary octyl phenol sulfide, calcium tertiary octyl phenol sulfide, barium-calcium tertiary octyl phenol sulfide, barium tertiary amyl phenol sulfide, calcium tertiary amyl phenol sulfide, barium nonyl phenol sulfide, etc. High alkalinity (i.e., high metal content) phenate sulfides are also included in the above description. These materials are prepared by reacting the phenol sulfide with an excess of metal base and then neutralizing the basic product, generally by CO<sub>2</sub> blowing.

The phosphosulfurized olefin materials are also well known in the art. These materials are prepared by reacting an olefin or an olefin polymer with  $P_2S_5$ . A specific material of this type used in an example of the invention was  $P_2S_5$  treated polybutene about 1100 molecular weight.

The products of the invention are prepared by forming the metal dithiophosphate in situ in oil in the presence of a detergent additive. This can be accomplished by a number of methods.

A preferred method is as follows:

(1) Form a first solution of the dithiophosphoric acid in a first oil-immiscible solvent, (2) form a second solution of a metal compound, capable of reacting with the dithiophosphoric acid to form the desired metal dithiophosphate, in a second oil-immiscible solvent which is preferably miscible with said first solvent, (3) slowly add the first and second solution simultaneously to oil containing the detergent while stirring to thereby slowly form metal dithiophosphate in the presence of said detergent, (4) separate the first and second oil-immiscible solvents from the oil mixture and (5) recover the resulting sol of metal dithiophosphate in oil. An illustration of the foregoing method is as follows: Dissolve the dialkyl dithiophosphoric acid in an alcoholic or aqueous solution. Form a second alcoholic or aqueous solution containing a salt of the desired metal, which salt is capable of reacting with the dithiophosphoric acid to form a metal salt of said dithiophosphoric acid. Simultaneously, the two solutions are added to an oil solution containing the detergent additive. A metal salt of the dialkyl dithiophosphoric acid will then be formed in situ in the presence of the detergent additive. The alcohol and oil will separate into an alcohol layer and an oily layer. The alcohol layer is decanted and the metal dialkyl dithiophosphate will be in a colloidal form in the oily layer protected by the detergent additive. The oily layer can be blown with nitrogen to remove any alcohol and finally the material can be heated under vacuum to remove any remaining volatile material. The material can also be filtered. If the material is very viscous, then hexane or a similar volatile diluent can be added to reduce the viscosity. The material is then filtered, and the diluent then volatilized. The final additive will be a stable colloidal sol of the metal dialkyl dithiophosphate and the detergent additive in oil. This additive can then be added to other oil compositions to thereby impart detergency, anti-wear and other desirable properties.

Alcohols which can be used are those which will dissolve the dithiophosphoric acid and the metal salt, and which are low molecular weight so as to be readily volatile. Such alcohols will include methyl, ethyl, n-propyl, isopropyl, etc. Alcohols are also preferred since they will readily separate from the oil-detergent mixtures and will not emulsify during mixing with the detergent.

The metal salts which are suitable for reaction with the dithiophosphoric acid are those which are soluble in the volatile alcohol and which also result in volatile acids when the metal is removed. Examples of such salts include acetates, chlorides, bromides, iodides, hypochlorites, etc.

While performed dialkyl dithiophosphoric acid can be used in carrying out the invention, said acid can be readily formed in situ in the low molecular weight alcohol. For example, alcohol is reacted with  $P_2S_5$  by simple heating to form the acid as is well known in the art. By using a large amount of the alcohol and a relatively small amount of the  $P_2S_5$ , then an alcohol solution of the dialkyl dithiophosphoric acid will result.

The final oil compositions of the invention will comprise a major proportion of lubricating oil, and 0.01 to 5.0 wt. percent of the metal dialkyl dithiophosphate and about 0.1 to 20 wt. percent of detergent additive (on an active ingredient basis). Preferred compositions will contain about 0.1 to 2.0 wt. percent of said dithiophosphate

and 1.0 to 10 wt. percent of detergent additive. Concentrates containing 10 to 70 wt. percent detergent additive and 2 to 14 wt. percent dithiophosphates, with the remainder oil, can also be prepared.

Various conventional lubricating oil additives may also be incorporated in the compositions of the invention to form finished lubricants. For example, additives in the amounts of .1 to 10 wt. percent each can be added, such as pour point dispersants, e.g. copolymers of vinyl acetate and alkyl fumarates; viscosity index (V.I.) improvers such as polyisobutylene and polymethacrylates; anti-oxidants such as alkyl phenols, bisphenols, sulfurized olefins; other detergents such as metal sulfonates or metal alkyl phenol sulfides, etc.

The invention will be further understood by reference to the following examples:

#### EXAMPLE I

*Solution A.*—A first alcohol solution was prepared by dissolving 0.5 gram mol of zinc acetate in methanol to form a total of 1,000 cc. of solution.

*Solution B.*—A second alcohol solution was prepared by reacting 0.5 gram mol of  $P_2S_5$  with 1000 cc. of 99% isopropyl alcohol, to form 1.0 gram mol of di-isopropyl dithiophosphoric acid in 1000 cc. of solution.

*Detergent additive.*—A lubricating oil detergent concentrate was used as a third component. This detergent consisted of about 70 wt. percent additive and about 30 wt. percent mineral lubricating oil. The additive itself was prepared by heating a mixture consisting of about 40 wt. percent of a phosphosulfurized isobutylene, 30 wt. percent of an oil concentrate of a high barium content tertiary octyl phenol sulfide and about 30 wt. percent of an oil solution containing 60 wt. percent of a high barium content sulfonate.

The phosphosulfurized polyisobutylene was prepared by reacting polyisobutylene of about 1100 molecular weight with 15 wt. percent based on the weight of polyisobutylene of  $P_2S_5$  at about 425° F. for about 8 hours under a nitrogen atmosphere. The oil concentrate of the barium tertiary octyl phenol sulfide consisted of about 43 wt. percent of said sulfide and about 57 wt. percent of a mineral lubricating oil. The barium tertiary octyl phenol sulfide was of the high alkalinity type having an alkaline neutralization number of about 90 and contained about 12 wt. percent barium. The high barium sulfonate had a barium content of about 14 wt. percent, based on the weight of the sulfonate. The sulfonic acid portion of the sulfonate was prepared by alkylating benzene with polypropylene, said sulfonic acid portion having an average molecular weight of about 440, and wherein 75 wt. percent of the sulfonic acid radicals had a molecular weight greater than 400. This sulfonate was prepared by reacting neutral barium sulfonate with additional barium hydroxide followed by neutralizing by bubbling carbon dioxide through the sulfonate.

Each of Solutions A and B was placed in a separate dropping funnel, and added slowly and simultaneously to 500 grams of detergent additive contained in a beaker, with constant stirring. After one hour all the ingredients were added and stirring was stopped. The mixture then separated into an oily layer and an alcohol layer. The alcohol layer was decanted and the remaining oily layer was heated to a temperature of about 225° F. and blown with nitrogen for about one hour in order to remove any remaining alcohol and acetic acid formed during the reaction. The material was next heated for about two hours in a vacuum oven at about 100° C. operating at a pressure of 150 mm. mercury to remove any remaining volatile material. The composition was then removed from the oven. This finished colloidal sol product analyzed 1.42% zinc, 1.96% phosphorus and 4.16% sulfur, and contained zinc diisopropyl dithiophosphate in a clear stable form.

## EXAMPLE II

*Solution C.*—44.4 grams of  $P_2S_5$  was added over a period of about half an hour to 200 grams of refluxing methanol, boiling at atmospheric pressure. A clear alcohol solution of dimethyl dithiophosphoric acid was thus formed.

*Solution D.*—22 grams of  $(CH_3COO)_2Zn \cdot 2H_2O$  was dissolved in 200 grams of methanol.

One-half of Solution C (containing 31.6 grams of dimethyl dithiophosphoric acid) was diluted with additional methanol to form a total of 250 cc. of solution. All of Solution B and all of said 250 cc. of solution of the dimethyl dithiophosphoric acid were simultaneously added from separate dropping funnels to 200 grams of detergent additive (same as in Example I) over a period of two hours and 40 minutes while vigorously stirring. Stirring was then stopped and the mixture was allowed to separate into an alcohol layer and an oily layer. The alcohol layer was decanted and discarded. The remaining oily bottom layer was then heated at 350° F. while stirring for a period of three hours while blowing nitrogen through said layer. Next, hexane was added to the oily layer to reduce its viscosity and the composition was filtered. The hexane was then stripped off by heating under vacuum. The remaining colloidal composition analyzed: 2.09 wt. percent zinc; 2.23 wt. percent phosphorus; 4.61 wt. percent barium and 3.06 wt. percent sulfur, containing zinc dimethyl dithiophosphate in a stable form.

## EXAMPLE III

*Solution E.*—The remaining half of Solution C from Example II was diluted with additional methanol to form a total of 250 cc. of solution.

*Solution F.*—37.9 grams of  $(CH_3COO)_2Pb \cdot 3H_2O$  were dissolved in water to form a total of 250 cc. of solution.

All of Solutions E and F were simultaneously added from separate dropping funnels to 200 grams of detergent additive (same as in Examples I and II), over a period of 2.5 hours while stirring at room temperature. After all of said Solutions E and F were added, the mixture was stirred for an additional hour. Stirring was then stopped and the mixture was heated to 100° F. The water layer, which separated, was siphoned from the mixture. The oily layer was heated to 225° F. while stirring and blowing with nitrogen until no more volatile material came off. The mixture was then cooled to room temperature and filtered to give a clear stable colloidal sol additive which analyzed 9.0 wt. percent lead and 4.77 wt. percent sulfur, containing lead dimethyl dithiophosphate.

## EXAMPLE IV

A lubricating oil composition was prepared by adding 4.7 vol. percent of the colloidal sol product of Example I to a multigrade SAE 10W-30 crankcase oil. The 55 crankcase oil consisted of a mineral base oil containing a polybutene viscosity index improver and a methacrylate viscosity index improver, and had a viscosity at 100° F. of 361.8 SSU, a viscosity at 210° F. of 69.7 SSU, and a viscosity index of 141.5.

The composition of Example IV above, was then subjected to a wear test in comparison with a similar lubricating oil composition containing the same viscosity index improvers, 4.0 vol. percent of detergent additive (same as in Example I), and 0.7 vol. percent of a commercial dialkyl dithiophosphate. The commercial dithiophosphate was a concentrate of 26 percent diluent oil and 74 volume percent of a zinc dialkyl dithiophosphate in which 65 percent of the alkyl groups were derived from  $C_6$  oxo alcohols and 35 percent were derived from isobutanol. The weight amount of the commercial zinc dialkyl dithiophosphate used in the comparison oil was equal to the weight amount of zinc dimethyl dithiophosphate in the composition of Example IV. Thus, the composition of Example IV and the comparison composi-

tion were comparable, but differing in the nature of the dithiophosphate.

The wear tests were run in a cam and tappet rig at temperatures in the range of 70° to 80° F. and spring pressures of 280 to 300 pounds. The cam and tappet rig consists of a small section of a Chevrolet V-8 engine block, including the front two camshaft bearing holders and the guides for four tappets, in which are mounted the front quarter of a camshaft and four tappets. Two frames for holding push rods and valve springs are mounted directly above the tappets in the normal V configuration. Provision is made for mounting two sets of springs, one above the other, if desired, to allow loadings up to about 700 pounds. Normal tappet loading for a 15 Chevrolet engine is about 225 pounds and runs up to about 425 pounds in some larger engines.

The bottom and ends of the block are closed with steel plates, forming a container for the test oil in which the camshaft and tappets are totally immersed. The hydraulic mechanisms are removed from the tappets, since 20 there is no oil pressure to operate them. The camshaft is driven by a two-horsepower electric motor at about 1740 r.p.m. Heat can be applied to the bottom by means of strip heaters, and cooling by water circulated through 25 the normal water jacket.

For studying normal wear, spring pressures of about 280 to 300 pounds have been found quite satisfactory, giving fairly sizable and reproducible wear in either 40 or 80 hour tests. The results obtained on oils of known 30 field performance rate the oils in their proper order. The tests are normally run at 70° to 80° F. using cooling water to carry off frictional heat, because this appears to be a somewhat more severe condition than higher temperature operation.

35 The results of the tests are given in Table I. They show that the additive of the present invention is much more effective than the commonly used commercial zinc dialkyl dithiophosphate, which has heretofore been considered the best available antiwear agent for crankcase 40 lubricant formulation.

Table I

| Lubricant                                                                                                  | Combined Cam and Tappet Wear in $10^{-4}$ Inch |          |
|------------------------------------------------------------------------------------------------------------|------------------------------------------------|----------|
|                                                                                                            | 40 Hours                                       | 80 Hours |
|                                                                                                            |                                                |          |
| Example IV Composition of Present Invention Composition Containing Commercial Zinc Dialkyl Dithiophosphate | 22.0                                           | 29.0     |
|                                                                                                            | 25.75                                          | 38.0     |

As demonstrated by the above table, the products of the invention are more effective than the best available prior art material of this nature. Furthermore, the sols of Examples I to IV were all stable, showing no separation upon standing.

The preceding examples are illustrative of the invention and other known detergent additives for motor oil can be utilized in forming the protective sol. For example, Example I can be repeated, but a  $P_2S_5$  treated polyisobutylene of the type previously described in said example is used as the suspending detergent in place of the detergent additive of Example I.

As still another example of the invention, Example I 65 is exactly repeated but in place of the 500 grams of detergent additive, 500 grams of a concentrate is used consisting of 40 weight percent of the neutral calcium salt of mono-dodecyl benzene sulfonic acid in 60 weight percent mineral lubricating oil. 5 wt. percent of the resulting colloidal sol product can then be added to 95 wt. percent of a mineral lubricating oil having a viscosity of 55 SUS at 210° F. to thereby improve the load-carrying and anti-wear properties of said lubricating oil.

In brief, the specific examples of detergents shown 75 represent preferred detergent materials, but any detergent

which will suspend the metal dialkyl dithiophosphate in a colloidal form in oil can be used.

What is claimed is:

1. An oil composition comprising a major amount of lubricating oil, about 0.1 to 20.0 wt. percent of a mineral lubricating oil detergent additive, and about 0.01 to 5.0 wt. percent of a metal dialkyl dithiophosphate, wherein each alkyl group has 1 to 3 carbon atoms and wherein said metal dialkyl dithiophosphate is water insoluble and is formed in the presence of said detergent additive. 5
2. An oil composition according to claim 1, wherein said detergent is an organic alkaline earth metal sulfonate.
3. An oil composition according to claim 1, wherein said detergent additive is a metal salt of an alkyl phenol sulfide.
4. An oil composition according to claim 1 wherein said detergent is phosphosulfurized polyisobutylene.
5. An oil composition as defined according to claim 1 wherein said metal is zinc.
6. An oil composition as defined according to claim 1 20 wherein said metal is lead.
7. A lubricating oil composition comprising a major amount of mineral lubricating oil, about 0.1 to 2.0 wt. percent of metal dialkyl dithiophosphate and about 1.0 to 10.0 wt. percent of a mineral lubricating oil detergent 25 additive wherein said metal dialkyl dithiophosphate is water insoluble and is prepared in the presence of said detergent additive by the reaction of dialkyl dithiophos-

phoric acid and a metal salt, and wherein each alkyl group contains 1 to 3 carbon atoms.

8. An oil concentrate consisting essentially of mineral lubricating oil, about 2 to 14 wt. percent of metal dialkyl dithiophosphate and about 10 to 70 wt. percent of a detergent additive, wherein said metal dialkyl dithiophosphate is water insoluble and is formed in the presence of said detergent additive by the reaction of a dialkyl dithiophosphoric acid and a metal salt, and wherein each alkyl group contains 1 to 3 carbon atoms. 10

9. An oil concentrate as defined according to claim 8 wherein said metal is zinc.

10. An oil concentrate as defined according to claim 8 wherein said metal is lead.

15

References Cited in the file of this patent

UNITED STATES PATENTS

|           |                       |               |
|-----------|-----------------------|---------------|
| 2,361,746 | Cook et al. -----     | Oct. 31, 1944 |
| 2,369,632 | Cook et al. -----     | Feb. 13, 1945 |
| 2,824,836 | Smith et al. -----    | Feb. 25, 1958 |
| 2,838,555 | Goldsmith -----       | June 10, 1958 |
| 2,956,018 | Carlyle et al. -----  | Oct. 11, 1960 |
| 3,018,247 | Anderson et al. ----- | Jan. 23, 1962 |

OTHER REFERENCES

Larson: "The Performance of Zinc Dithiophosphates as Lubricating Oil Additives" in Scientific Lubrication, August 1958. Page 15 relied on.